

## UNITED STATES PATENT OFFICE

2,111,203

## AMMUNITION

Willi Brün, Bridgeport, Conn., assignor to Remington Arms Company, Inc., a corporation of Delaware

No Drawing. Application May 28, 1934,  
Serial No. 727,151

6 Claims. (CL 52-2)

The present invention comprises the wholly novel concept of accelerating and controlling the performance of ammunition priming mixtures by the use of a substance or substances having catalytic properties.

The reaction of a priming mixture when struck a blow may be regarded as essentially the combustion of a fuel with a flame of substantial length and duration. The oxygen necessary for combustion is present in the form of a compound containing a substantial quantity of oxygen which becomes available for reaction with the fuel under proper conditions of temperature and pressure. The necessary conditions are produced by the decomposition of an explosive ingredient under the stimulus of a sharp blow. In priming mixtures of the past it has been necessary to carefully select and combine particular oxidizers, fuels and explosives, in order to insure certainty of combustion with the proper flame characteristics. The problem has been particularly difficult with the more stable non-corrosive oxidizers, such as barium nitrate, which yield their oxygen only at relatively high temperatures.

The discovery has now been made that the properties and combustion characteristics of priming mixtures can be improved and controlled by the introduction into the mixture of a small amount of one or more catalysts. Such catalysts may be either oxides or substances capable of oxidation. They are used in amounts of such small proportions that they cannot be considered themselves to enter into the reaction, either as oxidizers or as fuels; instead, they act as true catalysts, merely facilitating the reactions among other ingredients and probably themselves remaining substantially unchanged. The effect of the catalyst is such that in some instances the reaction temperature is substantially lowered.

A marked improvement in sensitiveness and powder igniting capacity of primers including such relatively sluggish oxidizers as barium nitrate has been effected by the use of catalysts. Their utility, however, is not limited to use in conjunction with any particular oxidizers, fuels, or explosives, or any particular combinations thereof. Suitable explosive or combustion initiating and sensitizing ingredients include such substances as lead styphnate, diazodinitrophenol, mercury fulminate, normal and basic lead azide, basic lead picrate, the lead salts of di- and tri-nitro benzol, the lead salts of dinitro-ortho cresol, the lead salts of dinitrosalicylic acid, tetrazene and its salts, the salts of nitro-tetrazole, azo

tetrazole and diazo-amino-tetrazole, lead hypophosphite, and lead dinitro-phenyl azide.

Suitable oxidizing ingredients include one or more of the usual chlorates, perchlorates, nitrates, chromates, permanganates and peroxides.

Suitable fuels include antimony sulphide, lead sulphocyanate, calcium silicide, ferro-silicon, and potassium ferrocyanide. Many of the aforementioned combustion initiating and sensitizing ingredients likewise react as fuels.

The field of useful catalysts includes generally the metals, metallic alloys and oxides, and the salts of acids having radicals, usually complex, which contain metals. Such acids will be called "metallo" acids. The metals which either alone or in their oxides and alloys are primer catalysts include copper, silver, gold, aluminum, zirconium, tin, lead, antimony, bismuth, zinc, vanadium, chromium, molybdenum, tungsten, manganese, iron, cobalt, nickel, palladium and platinum. The salts include potassium dichromate, sodium tungstate, potassium stannate, and mercuric chromate. The presence of even minute quantities of such catalysts has been found to be very beneficial. It is impracticable to specify the minimum amount of catalyst that will give the desired results, owing both to substantial variations among different catalysts and to the difficulty of securing uniform distribution of very small percentages of one solid material throughout a mixture of other solid materials. It may be said, however, that the optimum amount of catalyst rarely exceeds 2% and ordinarily does not exceed 1% of the entire mixture. Larger quantities of certain catalysts, for example the oxides of cobalt, have been found to actually deaden a mixture, rendering it less sensitive to blow.

A typical mixture comprises suitable proportions of tetrazene, lead styphnate, barium nitrate, lead sulphocyanate and glass, with up to about 1% of such a catalyst as platinum, silver, bismuth, bismuth trioxide, manganese dioxide, cobaltic oxide, cobaltous oxide or sodium tungstate. The catalyst increases both the sensitiveness and the powder igniting capacity of the mixture without undesirable effects on its other properties. This mixture, however, is merely typical. Catalysts have been found to be applicable to priming mixtures generally, and the appended claims are to be broadly construed.

What is claimed is:

1. A priming mixture containing a fuel ingredient, a combustion initiating explosive, an oxidizing ingredient consisting essentially of barium

nitrate, and not over 2% of a catalyst having the property of accelerating and lowering the temperature of reaction between the barium nitrate and the fuel, said catalyst being selected from 5 the group consisting of the metals, mixtures and alloys of the metals, the metallic oxides, and the salts of the metallo acids.

2. A priming mixture containing a fuel ingredient, a combustion initiating explosive, an oxidizing salt, and a small percentage of a catalyst having the property of accelerating the reaction 10 between the oxidizing salt and the fuel, said catalyst being an oxide of bismuth.

3. A priming mixture containing a fuel ingredient, an oxidizing ingredient, and an oxide of bismuth.

4. A priming mixture containing a fuel ingredient, an oxidizing ingredient, and a small per-

centage of a catalyst having the property of accelerating the reaction between the oxidizing ingredient and the fuel ingredient, said catalyst being a finely divided metal.

5. A priming mixture containing a fuel ingredient, an oxidizing ingredient, and a small percentage of a catalyst having the property of accelerating the reaction between the oxidizing ingredient and the fuel ingredient, said catalyst comprising finely pulverized silver. 5

6. A priming mixture containing a fuel ingredient, an oxidizing ingredient, and a small percentage of a catalyst having the property of accelerating the reaction between the oxidizing ingredient and the fuel ingredient, said catalyst 10 comprising finely pulverized lead. 15

WILLI BRÜN.